

## UNITED STATES PATENT OFFICE

BENNO HOMOLKA, DECEASED, LATE OF FRANKFORT-ON-THE-MAIN, GERMANY; BY RUDOLF ROSENTHAL, EXECUTOR, OF FRANKFORT-ON-THE-MAIN, GERMANY, AS- SIGNOR TO I. G. FARBENINDUSTRIE AKTIENGESELLSCHAFT, OF FRANKFORT-ON- THE-MAIN, GERMANY, A CORPORATION OF GERMANY

PROCESS OF DESENSITIZING SILVER-BROMIDE EMULSIONS AND PLATES OR FILMS COVERED WITH SUCH EMULSIONS

No Drawing. Application filed December 20, 1927, Serial No. 241,447, and in Germany June 15, 1927.

The present invention relates to a process of desensitizing silver bromide emulsions and plates or films covered with such emulsions.

5 It is known that dyestuffs of the group of the safranines of the general formula:



10

15 in which Ac means the residue of an acid, that is to say 3-6-diamino-phenyl-phenazonium salts, for instance the pheno-safranine and tolu-safranine, have the property of de- sensitizing photographic silver-bromide 20 emulsions in such a degree that they can be developed in yellow light. The said dye- stuffs have, however, the disadvantage that they stain the gelatin layer of the plates and 25 films, the vessels and also the fingers and clothes of the operators, intensely red. Though in the case of photographic plates this color can be removed from their gelatin layer, this cannot be done with films, be- 30 cause the latter, when treated with safranine dyestuffs, are stained so much that they are entirely spoiled thereby and rendered unfit for use. For this reason the process of de- sensitizing by means of safranines cannot be 35 applied in developing films.

The inventor has now found that the isom- erides of the said safranine dyestuffs in which at least two amino groups are situated in one and the same carbon nucleus belonging 40 to the azine complex, have a very strong de- sensitizing action upon photographic silver bromide emulsions. These compounds offer the advantage over the normal safranine dyestuffs that, in spite of their pronounced 45 dyestuff character, they do not stain at all,

or only very slightly, the gelatin layers, the fingers of the operator etc., so that the films or other materials are not spoiled, and the slight coloring imparted to them can be easily washed out by means of water. For instance 50 the following compounds of the said kind are suitable for producing this effect:

The 1-3-diamino-phenyl-phenazonium salts of the formula:



55

60

65

in which Ac represents the residue of an acid (see Berichte der Deutschen Chem. Ges. Vol. 33 page 3074); the 2-3-diamino-phenyl-phenazonium salts of the formula:



70

75

in which Ac represents the residue of an acid 80 (see Helvetica Chimica Acta VIII page 279) and also the homologues and substitution products thereof, for instance the alkyl-, halo- gen-, amino-oxyalkyl derivatives or the like.

The photographic layers may be desensi- tized either by immersing the plates or films, before they are developed, for 1-2 minutes into the solution of the iso-diamino-phenyl-phenazonium salt or by adding a small quantity of this compound to the developer. 90

The following examples serve to illustrate the invention but they are not intended to limit it thereto.

1. The plate or film to be developed is immersed into an aqueous solution (about 1:5000) of 1-3-diamino-phenyl-phenazonium-chloride for about 1-2 minutes and the development can then be effected in yellow light or in candle light.

10 2. About 100 ccm. of the developer are mixed with 2 ccm. of a solution (1:500) of 1-3-diamino-phenyl-phenazonium-chloride. After the plate of the film has remained in the developer for about one minute, the development can be finished in yellow light or candle light.

15 3. In the processes set forth in (Example 1) and (Example 2) there may be used instead of the above named compound, for instance the following compounds: 1-3-diamino-7-aminophenyl-phenazonium-chloride; 2-3-diamino-phenyl-phenazonium-nitrate; 1-3-diamino-6-(or 7)-chlorphenyl-phenazonium-chloride; 1-3-diamino-ortho-(or para)-25 tolyl-phenazonium-chloride of the following formula:



40 1-3-diamino-ortho-(or para)-oxyalkyl-phenyl-phenazonium-chloride; 1-3-diamino-6-oxyalkyl-phenyl-phenazonium-chloride of the formula:



55 What is claimed is:

1. The process of desensitizing photographic silver-bromide layers, which consists in treating the layer with an amine of a phenylphenazonium salt in which at least 60 two amino groups are situated in one and the same carbon ring belonging to the azine complex.

2. The process of desensitizing photographic silver-bromide layers, which consists



wherein X represents hydrogen or any substituent and Ac the residue of an acid.

3. The process of desensitizing photographic silver-bromide layers, which consists in treating the layer with a salt of the following constitution:



95

In testimony whereof, I affix my signature.

RUDOLF ROSENTHAL,  
Executor of the Estate of Benno Homolka,  
Deceased.

100

105

110

115

120

13